

Aug. 25, 1953

D. T. TARR, JR., ET AL  
TREATING ARSENICAL GOLD ORES

2,650,159

Filed Nov. 23, 1949

2 Sheets-Sheet 1



FIG. I.

INVENTORS:  
FRANCOIS A. FISCHER &  
DONALD T. TARR, JR.  
BY

Arthur Middleton  
ATTORNEY

Aug. 25, 1953

D. T. TARR, JR., ET AL  
TREATING ARSENICAL GOLD ORES

2,650,159

Filed Nov. 23, 1949

2 Sheets-Sheet 2



**INVENTORS:**  
**FRANCOIS A. FISCHER &**  
**DONALD T. TARR, JR.**  
**BY**

BY *Arthur Nidolson*  
ATTORNEY

## UNITED STATES PATENT OFFICE

2,650,159

## TREATING ARSENICAL GOLD ORES

Donald T. Tarr, Jr., Denver, Colo., and Francois A. Fischer, Brussels, Belgium, assignors to The Dorr Company, Stamford, Conn., a corporation of Delaware

Application November 23, 1949, Serial No. 128,962

2 Claims. (Cl. 75—69)

1

This invention relates to the roasting of arsenopyrite ores and particularly to the roasting of those gold bearing arsenopyrite ores which contain commercially significant amounts of gold in association with the mineral arsenopyrite.

A gold bearing ore consisting essentially of arsenopyrite, pyrite, stibnite, with lesser amounts of other sulfide materials, together with such gangue or rock minerals as carbonates of lime, magnesia, etc., with quartz was used for the experimentation leading to the invention disclosed herein. This type of arseno-pyrite gold bearing ore contains its gold values in several forms. There is present so-called free gold which may be recovered by any of the usual methods of chemical or mechanical concentration. In addition to this free gold there is a commercially valuable quantity of gold which is not responsive to ordinary means of recovery. Attempts have been made to recover this gold by roasting methods followed by cyaniding the roasted ore. But, heretofore, in attempting to recover these normally unavailable gold values, processes have been developed which might be characterized by the fact that, in general, they require large complex equipment involving a high initial installation cost; also, because of the wasteful method of burning the sulfides, at certain portions of these old processes, extraneous fuel must be added because the ore at those points becomes no longer self-roasting. Because of these factors, many gold ores which contain small quantities of gold, or many gold ore tailings, no longer become economically feasible to work and must be rejected. This is particularly true of low-sulfide ores which are not self-sustaining and which require the expensive application of extraneous fuel.

In order to recover these unrecoverable gold values it is necessary to release them from their original combination in the ore and thus make them amenable to cyaniding. To so release them the ore must be roasted so that every particle is fractured. It must be a complete roast, i. e., one containing no residual unconverted mineral still present in its original, natural state of chemical combination.

If the ore is not completely roasted, then ferrous iron will be present in the final product and this iron will be a large consumer of cyanide, otherwise known as a cyanide. If the amount of cyanide is high, then the cyanide consumption is increased and the economic worth of the process is serious jeopardized. Thus the ore must be completely roasted, resulting in the conversion of the ferrous iron to the ferric state, in which state it is not detrimental.

2

However, when the ore is completely roasted, the arsenic is converted to its highest oxidation state, namely,  $As_2O_5$ , in which form it is not volatile. Thus it remains behind in the ore and serves to plug the pores, preventing cyanide solution from reaching the entrapped gold values.

Thus the problem resolves itself to one in which there must be a completely roasted ore and yet which must not contain  $As_2O_5$ , which in itself is the necessary product of a complete oxidation or roast.

The roasting of arsenopyrite gold ores in conventional equipment using conventional means is known and in these processes, oxidation of elements originally present in mineral arsenopyrite and associated oxidizable minerals may be carried substantially to completion.

By using conventional equipment, the color of the roasted product is known to vary from black to red, but operators report that the red roast is the highly desirable one because ferrous iron is absent.

In these processes, because of the poor control over both oxygen input and roasting temperatures, these undesirable oxidation products appear in the roast, which products are high in cyanide consumption, with the result that the processes become further economically unsound.

It is then an object of this invention to produce a substantially completely roasted gold-bearing arsenopyritic ore in such a manner as to make possible the subsequent substantially complete recovery of all the gold values from the roasted ore by cyanidation. It is another object of this invention to recover the gold with an minimum consumption of cyanide so as to make the process commercially feasible. It is a further object to discover a means of controlling the color of the roasted product so as to obtain this highly desirable red roast yielding high gold recovery. And it is yet another object to develop a process which will utilize the latent sulfide heat-generating properties of gold ores, particularly low sulfide ores, to their utmost so that no fuel need be added to obtain a completely roasted product from these low sulfide ores.

These objects are attainable by roasting the ore under fluidizing conditions in two stages with carefully controlled oxygen furnished to the ore during roasting in each stage, whereby the arsenic compounds are substantially removed and the ultimate product will be amenable to high gold recovery, will be the desirable red color, and will be completely roasted.

Before presenting a detailed description of apparatus and process constituting the invention

## 3

hereof, it is important to note that according to this invention the roasting of ore is accomplished in a fluidizing furnace or reactor in which the ore is in a fluidized condition.

A fluidized solids reactor or roaster or furnace in its most simple form is a vertical vessel having a perforated horizontal partition in its lower portion. Finely divided solids are supplied to the vessel above the partition by a conduit and gas is passed upwardly from the bottom of the vessel through the partition and through the powdered solids. The gas passes through the solids at such a rate that the solids are kept as a suspended bed or layer in the vessel. The solids are in dense, turbulent suspension and are usually referred to as a fluidized bed.

A fluidized bed is a very dense suspension of fine solids in a supporting flowing gas. The density or solids-concentration per unit volume of such a fluidized bed is very high, being commonly of the order of 10 to 100 pounds of solids per cubic foot of bed volume. This bed density is to be contrasted with typical dilute dispersions or suspensions, such as dusty air wherein the density of solids concentration is of the order of only  $\frac{1}{50}$  of a pound per cubic foot of the dispersion. In addition, the solid particles of a fluidized bed are in a high state of turbulence or erratic, zig-zag motion in the bed even when the suspending gas velocity is quite low; this high turbulence causes intimate and rapid mixing of the solids particles so that in a typical bed complete mixing of the solids appears to take place instantaneously. A fluidized bed, because of its high density and great turbulence, is noted for the rapid transfer of heat between its solid and gaseous components; this heat transfer is so rapid that a remarkable uniformity or homogeneity in the temperature of the bed results.

In some detail, a fluidized solids reactor consists essentially of a gas-tight chamber closed at the bottom with a plate perforated to permit upflow and secure uniform flow-distribution of gases admitted to a windbox below the plate; means for admission of sub-divided material to be roasted, and means for removal of roasted material as well as means for removal from the reactor of the gas after it is reacted with fluidized particles therein. The gas passes into the windbox, thence upwardly through the perforated plate, (hereafter referred to as the constriction plate) and through a mass of the finely divided solids to be roasted. The velocity of the gas through the mass or layer or bed of finely divided solids (hereafter referred to as the fluidized bed) is controlled so that it suffices to produce an exceedingly turbulent agitation of the solids through which the gas is passing and which by its passage are densely suspended and, in general, caused to behave like a boiling liquid including being capable of presenting a fluid-level. This velocity, as measured in the upper portion of the reactor above the level of the densely suspended solids, is commonly of the order of 0.2 to 2.0 feet per second, and is referred to as superficial velocity. The velocity of the gas, while it is essential that it be in a range sufficient to "fluidize" the fuel solids, must be below the rate at which all or substantially all of the solids suspended would be entrained and carried quickly out of the reactor as a dispersed or dilute suspension in the exit gas. Such a dispersed suspension behaves substantially like the exit gas and is unlike the fluidized bed. The means for removal of roasted solids from the reactor will

## 4

usually comprise a vertical or steeply inclined conduit leading outside the reactor and provided with means for permitting a free discharge of the solids but not a free discharge of gases from the chamber. The minimum depth of the fluidized bed of solids within the reactor may be determined by the elevation of the discharge means as measured upward from the constriction plate. The depth will commonly be of the order of 1 to 5 feet.

The approximate fluidizing velocity, the best depth of the fluidized bed, temperature control methods and other conditions of operation hereinafter referred to, which give the best results, may be determined by preliminary test on the particular ore which is to be roasted by our process.

According to this invention, therefore, the roasting of the arseno-pyrite ore is carried out in an apparatus which permits accurate regulation of conditions affecting the quality of the roasted ores. The conditions in the reactor may be readily determined at any time and adjusted as required or the operations of the roasting apparatus may be automatically regulated within desired limits, as we shall subsequently disclose.

In roasting an arsenopyritic gold bearing ore by our process, finely divided particles of the ore are introduced to the upper bed in the primary zone of the reactor above the apertured constriction plate and a free oxygen-bearing gas is up-flowed through the constriction plate at a rate sufficient to maintain the ore particles in a violent, turbulent, mobilized condition of dense fluidized suspension. The bed of mobilized or fluidized ore will act like a liquid in that it is capable of presenting a level, will flow like a liquid under hydraulic head and, most pertinently, will have substantially homogeneous temperature conditions throughout the bed depth. The oxygen bearing gas must satisfy the dual requirement of being supplied at a rate sufficient to maintain the particles in a fluidized state and containing a sufficient quantity of oxygen to controlledly oxidize the ore to the proper degree which this invention teaches.

This partially oxidized ore then flows to the lower bed in the secondary zone where in the carefully controlled oxygen-bearing gas again fluidizes it and completes the roasting or oxidation of the sulfidic constituents. The product is removed from this second bed by a downwardly slanting pipe, the height of the upper end of which controls the level of the bed. This product has been discovered to be substantially completely roasted, is the desirable red color, and will give a high gold recovery with low cyanide consumption.

The novel features of this invention will be understood and more fully appreciated from the following description, particularly when considered in connection with the accompanying drawings.

In the drawings, Figure 1 is a simplified flow sheet or scheme of the progress of the materials through the roasting operation. Figure 2 is a vertical sectional view of a roasting apparatus of fluidized solids type reactor suitable for performing the two bed embodiment of invention and wherein and by which the invention may be commercially realized.

More particularly, Figure 1 shows the ore feed entering bed 17, passing down the downcomer 19 into bed 18. After roasting, the ore product is removed through conduit 29. The legends

show chiefly the reactions, temperatures and products in the process.

In Figure 2, there is shown a vertical cylindrical reactor collectively designated 11 which has a detachable top member 13, a detachable bottom member 14 and side walls 12. Internally, the vessel 11 is lined with refractory brick 15, has two horizontal apertured partitions 31 and 33 therein which are each adapted to support fluidized beds 17 and 18 respectively, and has a horizontal gas impermeable partition 81 to separate the two zones. The primary treatment zone P is the portion of the reactor 11 occupied by bed 17; the secondary treatment zone S is the portion of reactor 11 occupied by bed 18. Downcomer 19 leads from the surface level of bed 17 to a point below the surface level of bed 18 and serves to conduct treated solids in bed 17 to bed 18. In this particular embodiment, the upper end of downcomer 19 also serves to determine the level or height of bed 17. Above bed 17 is freeboard zone 27 and above bed 18 is freeboard zone 20. Fine solid particles of metallurgical sulfides are supplied to top bed 17 by means of a screw-conveyor 42 in casing 45, which in turn is supplied by hopper 43. The conveyor 42 is driven by motor 44. Gas for fluidizing and treating the solids in beds 17 and 18 is supplied to the lower portion of vessel 11 by means of conduit 40 and the rate thereof controlled by valve 41. The treatment gas passing through conduit 40 enters wind-box 22, rises through the apertures 23 of horizontal partition 33 and enters bed 18. After fluidizing bed 18, the gas rises through freeboard zone 20 and passes through conduit 50 into cyclone 51 wherein the fines which were carried along in the gas stream are separated. These fines frequently represent completely roasted finished product and as such would be drawn off through conduit 52, controlled by valve 53. The treatment gas leaving cyclone 51 passes through conduit 54 into wind box 55, passes upward through apertures 25 of horizontal partition 31 to bed 17. From bed 17, the gas flows up through freeboard zone 27, leaves reactor 11 by means of conduit 10, passing through cyclone separator 36. The gas then leaves cyclone 36 by means of conduit 56 and the solid partially roasted fines drop down conduit 57, controlled by valve 60, into bed 17, entering below the bed level, wherein they become completely roasted.

In starting up the process as depicted in Figure 2, air under controlled pressure is supplied to vessel 11 through conduit 40. To this is added fuel such as natural gas which is ignited within vessel 11 and serves to preheat it. Alternatively, liquid fuel may be supplied by pipe 70. Inert material, such as sand, or roasted tailings, is fed into both beds so as to form an air resistor and also to cover the lower end of downcomer 19 to prevent short circuiting of influent air. It has been found that the height and length of the downcomer 19 must be so determined that the weight of the solids therein will be sufficient to overcome the gas pressure in the secondary zone, so as to prevent this short-circuiting of the gas up the downcomer. Bed 17 may be supplied with the above mentioned inert material by screw-conveyor 42; bed 18 may be so supplied by blowing the material back up outlet pipe 29. When the vessel 11 is up to a sulfide oxidizing temperature of about 800° C., fine metallurgical solid sulfide particles are supplied to bed 17 by screw-conveyor 42. These ores become self-roasting exothermally and the auxiliary fuel sup-

ply may now be shut down. Gradually the level of fluidized solids in bed 17 builds up until the inlet level of downcomer 19 is reached, whereupon partially roasted solids flow down the downcomer 19 to a point above partition 33 but below the upper end of takeoff conduit 29. These solids accumulate in fluidized state until their level reaches the upper end of conduit 29 whereupon they flow, controlled by valve 38, to a point outside reactor 11 where they are cyanided or otherwise treated for recovery of their gold values by methods beyond the scope of this invention.

Before describing the practical operation of our process it might prove helpful to define the term "theoretical oxygen" as used therein. By theoretical oxygen is meant that quantity of oxygen which will be stoichiometrically capable of converting Fe into  $Fe_2O_3$ , S into  $SO_2$ , As to  $As_2O_3$  and M into  $MO_2$ .

We have determined and demonstrated that the practical and commercial mode of practicing our invention is substantially as follows. The starting ores which were used are demonstrated below.

| Sample # | Fe      | S       | As      | Sb      | Au      |
|----------|---------|---------|---------|---------|---------|
|          | Percent | Percent | Percent | Percent | Oz./ton |
| 1        | 21.9    | 17.1    | 14.7    | 0.77    | 4.26    |
| 2        | 22.75   | 18.6    | 4.95    | 0.07    | 1.2     |
| 3        | 13.5    | 14.5    | 1.9     | 0.05    | 0.98    |

It is to be noted in these samples that the arsenic and gold values vary over a wide range and that the sulfur value is, in general, fairly low. In terms of old processes, the sulfur value of sample #3 may be said to be in the range in which the ores would not be self-roasting without extraneous fuel.

After the process has undergone the starting up procedure, as previously outlined, the oxygen bearing gas is fed to the primary zone so that, arbitrarily, it contains only 50% of theoretical oxygen. Necessarily included in the gas will be the volatile products from the secondary zone, the principal constituent of which is sulfur dioxide. By supplying 50% of theoretical oxygen it is believed that arsenic trioxide and/or arsenic sulfide ( $As_2S_2$ ) is formed in this zone and then the arsenic fumes off at the operating temperatures suggested, thus effectively removing the arsenic from the ore. This figure is selected only for convenient operation and it has been found that any amount short of 100% of theoretical oxygen may be supplied, just so long as substantially no free oxygen is found in the exiting gas. If free oxygen is found, then the feed rate of the ore is increased so as to consume this oxygen. Normally, the ore feed rate is adjusted so as to give the ore a total residence time of 18 hours in the reactors. Using 50% of theoretical oxygen, and at a bed temperature of 505° C., it was discovered that 60% of the arsenic was eliminated. Maintaining the same oxygen input, but raising the temperature of the bed in the primary zone to 550° C., proved that 94% of the arsenic was eliminated.

This substantially arsenic free ore now flowed down to the secondary zone. The sulfur content at this point was about 50% of the original sulfur content of the ore. Air was passed through this secondary zone at such a rate that it contained 150% of the theoretical requirement. The temperature was found to be optimum at 625° C. However, since a fully roasted product is desired here, the temperature may be permitted to vary

so as to accomplish this. The limiting range of temperature is the fusion point of the material in the condition in which it comes from the primary zone. Slight amounts of impurities, such as lead, will cause this temperature to vary. The material must not be permitted to fuse, however, as this condition is anathema to fluidizing media and a dead bed will result. From a practical operating point of view, if the temperature of the secondary or lower bed is noticed decreasing it means that the oxygen in the upper bed is nearing 100% of theoretical and consuming nearly all of the sulfur in the upper bed, thus permitting very little of it to come through to the lower bed to be consumed. Under these circumstances, if the ore feed rate is increased, with oxygen remaining constant, it will result in the ore leaving the primary zone having a higher sulfur content. The roasting temperature of the lower zone will then be seen to increase. Thus a very fine control over the reaction may be obtained at all times and the low-sulfur ores may always be maintained as self-roasting in both zones.

If the temperature tends to run away at any time, water sprays 72 are provided to control it and prevent fusion of the material.

When arsenopyritic gold bearing ore is subjected to the process described in this invention, it will always be recovered from the reactor as a red calcine, indicating a complete roast. When this red calcine is subjected to cyanidation to remove the gold, approximately 93% of the gold is extracted. The amount of cyanide necessary to obtain this high gold recovery is approximately 2-3 lbs. per ton of ore, and the process becomes economically feasible. With the apparatus herein described, this process is capable of close control as regards temperature, feed and influent oxygen yielding in a self-sustaining roasting operation a product from which the gold recovery becomes economically feasible.

It is also within the ambit of this invention to supply fuel to the fluidized bed for those ores whose sulfur value is so low that even with this process they are not self-roasting. By so supplying fuel to the bed, it will be caused to burn directly in the bed itself and thus its maximum heat value will be utilized. Coupling this with the efficient complete use of the heat furnished from any sulfur available, gives a process which can readily be seen to be usable for the poorest of ores.

We claim:

1. The continuous process for roasting finely-divided gold-bearing arsenopyrite solids to render their gold values amenable to cyanidation with

minimum cyanide consumption, comprising the steps of establishing and maintaining a fluidized treatment bed of such solids in a primary treatment zone by feeding solids thereto and passing therethrough at solids fluidizing velocities an uprising stream of free-oxygen bearing gas while maintaining the solids at roasting temperatures less than fusion temperatures, and under such conditions effecting substantial removal of arsenic as volatile arsenic compounds to yield partially roasted arsenic-free solids by regulating the quantity of free-oxygen in the uprising gas stream to be an amount sufficient to oxidize a portion of the sulfide-sulfur content of the solids to sulfur-dioxide but insufficient to so oxidize all of such sulfur, discharging gases including volatile arsenic compounds from the bed and from the zone, discharging partially roasted arsenic-free solids from the primary zone to a secondary zone to establish in the latter zone a bed of such solids, treating solids of the latter bed under solids fluidizing conditions to yield substantially completely roasted solids by maintaining the bed at roasting temperatures less than fusion temperatures while passing therethrough at solids fluidizing velocities an uprising stream of gas initially containing free-oxygen in an amount at least sufficient to substantially oxidize all residual unoxidized oxidizable constituents of the bed solids, discharging gases from the zone, and discharging substantially oxidized arsenic-free solids from the zone.

2. The process according to claim 1 wherein the quantity of free-oxygen supplied to the secondary treatment zone is sufficient so that gases discharged from that zone contain residual free-oxygen in an amount sufficient to oxidize to sulfur-dioxide at least a portion of the sulfide-sulfur content of the bed solids in the primary treatment zone but insufficient to oxidize all of such sulfur to sulfur-dioxide, and the free-oxygen bearing gases supplied to the primary zone comprise the gases discharged from the second zone.

DONALD T. TARR, JR.  
FRANÇOIS A. FISCHER.

References Cited in the file of this patent

UNITED STATES PATENTS

| 50 | Number    | Name         | Date          |
|----|-----------|--------------|---------------|
|    | 1,941,592 | Bacon et al. | Jan. 2, 1934  |
|    | 2,444,990 | Hemminger    | July 13, 1948 |

OTHER REFERENCES

- 55 "Canadian Mining and Metallurgical Bulletin,"  
April, 1949, pages 178-187.  
"Chemical Engineering," Dec., 1947, page 114.